

# United States Patent Office

2,732,303

Patented Jan. 24, 1956

1

2,732,303

## ANTIFOGGING AND HARDENING AGENTS FOR PHOTOGRAPHIC EMULSIONS

John Morgan and Donald Arthur John Starkey, Harrow, England, assignors to Eastman Kodak Company, Rochester, N. Y., a corporation of New Jersey

No Drawing. Application September 16, 1953,  
Serial No. 380,586

13 Claims. (Cl. 95—7)

This invention relates to compounds useful as fog-inhibiting agents or hardening agents for photographic emulsions, and to photographic emulsions containing them.

It is well known that photographic emulsions on storage tend to lose sensitivity and to become spontaneously developable without exposure to light. There is normally a detectable amount of the silver salt reduced during development in the areas where no exposure was given; this is commonly called "fog," and sometimes called "chemical fog" where it is necessary to distinguish between it and the effects of accidental exposure to radiation; in this invention, we are not concerned with the latter.

Fog depends both on the emulsion and the conditions of development; for a given emulsion it increases with the degree of development. With constant development conditions, it tends to increase with time, temperature and relative humidity of storage conditions; it is common practice to make accelerated tests of the stability of photographic emulsions by storage at increased temperature or humidity, or both. It is of course desirable to have emulsions as stable as possible under the conditions of high temperature and humidity which may occur in tropical climates, for example. Fog usually appears over the whole area of the sensitive coating, but when severe, it frequently is non-uniform. Fog may also be caused by exposure to chemicals, for example, hydrogen sulfide and other reactive sulfur compounds, hydrogen peroxide vapor, and strongly reducing materials. While antifoggants and stabilizers may protect, to some extent, against such effects, it is normally understood that an antifoggant protects against spontaneous growth of fog during prolonged storage or storage at high temperatures and humidities, or during development to maximum contrast and speed, or both.

It is, accordingly, an object of our invention to provide a method for stabilizing photographic emulsions. A further object of our invention is to provide a method for hardening photographic emulsions. Another object of our invention is to maintain the sensitivity and fog of silver halide emulsions at or close to initial optimum values under keeping conditions of high temperature and humidity. A further object is to provide photographic silver halide emulsions containing antifoggants (or stabilizers) or hardening agents. Other objects will become apparent from a consideration of the following description and examples.

The above objects are, in general, accomplished by adding to the photographic emulsions at least one compound selected from those represented by the following two general formulas:

(1)



and

(2)



wherein R represents a halogenoalkyl group, such as

2

chloromethyl, bromomethyl, iodomethyl, dichloromethyl, dibromomethyl, diiodomethyl, trichloromethyl, tribromomethyl, triiodomethyl,  $\alpha$ -chloroethyl,  $\beta$ -chloroethyl,  $\alpha$ -bromomethyl,  $\beta$ -bromomethyl,  $\beta$ -idoethyl, etc. In the compounds selected from those represented by Formula 2, the R group can be the same or different.

The compounds selected from those represented by Formulas 1 and 2 above are, in general, known compounds. The compounds represented by Formula 1 above can advantageously be prepared by reacting a halogenated aliphatic carboxylic acid together with ethylene oxide in varying amounts. By varying the quantity of ethylene oxide, it is possible to produce monoesters wherein n has any desirable value. Accordingly, n can represent any positive integer, e. g., 1 to 200, or more. This method of making monoesters is well known and has been previously described in the prior art. Advantageously, the reaction is carried out in the presence of an acidic catalyst, such as boron trifluoride (generally in the form of a complex, such as with acetic acid, diethyl ether, etc.).

The compounds embraced by Formula 2 above can advantageously be prepared by reacting together an acid halide (e. g. chloride, etc.) of a halogenated aliphatic carboxylic acid with a suitable glycol, such as ethylene glycol, diethylene glycol, triethylene glycol, the polyethylene glycols, etc. Thus, in Formula 2 above n can also represent any positive integer, e. g. 1 to 200 or more. The condensations can advantageously be carried out in the presence of an acid-bonding agent, such as pyridine, quinoline, etc., although such acid-bonding agents need not be employed unless so desired. Also, if desired, an inert solvent, such as dioxane, diethyl ether, etc., can be employed.

Alternatively, the compounds of Formula 2 can be prepared by heating together, in the presence of an acid esterification catalyst, a glycol, such as those listed above, with a halogenated aliphatic carboxylic acid. Suitable esterification catalysts comprises sulphuric acid, p-toluenesulphonic acid, etc. The speed of the esterification can be increased through the use of water-entraining agent, such as benzene, toluene, etc., which can be azeotropically distilled off.

When employing higher molecular weight glycols in the methods outlined above, a mixture of esters generally results. For example, when a large amount of ethylene oxide is employed with respect to the quantity of halogenated aliphatic carboxylic acid, the reaction mixture contains a mixture of esters wherein the value of n in Formula 1 varies. Likewise, when a polyglycol is reacted with a halogenated aliphatic carboxylic acid or carboxylic halide, a mixture of diesters wherein the value of n varies, results. While it is sometimes possible to separate these mixtures into the component esters, it is not necessary to do so. Accordingly, in the table given below, in some cases only the average value of n is set forth. Mixtures of esters, or pure esters, can be employed to advantage in practicing our invention. Mixtures of monoesters with diesters are also effective.

The following examples will serve to illustrate methods of preparing certain of the esters useful in our invention.

### Example 1.—Triethyleneglycol-bis (chloracetate)

Triethylene glycol (30 gms. 0.2 mol.) was cooled to 0° C. in an ice-bath and redistilled chloracetyl chloride (54 gms. 0.48 mol.) added slowly with stirring. The temperature was kept below 20° C. during the addition, which was complete in about 20 mins. The solution was stirred for a further 30 minutes and the excess acid chloride removed by heating on the steam-bath at water-pump pressure. The viscous oil was distilled. B. P. 228°—230° C./20 mm., yield 55 gms. (91% theoretical).

*Example 2.—Triethyleneglycol-bis (β-chloropropionate)*

Triethylene glycol (15 gms. 0.1 mol.), β-chloropropionic acid (23 gms. 0.11 mol.) and p-toluenesulphonic acid (0.5 gms.) were azeotropically refluxed in benzene (250 ml.) for 16 hours and 4.5 ml. of water collected. The benzene was removed and the clear oil distilled. B. P. 216° C./15 mm. yield = 17 gms. (52%).

*Example 3.—Polyethyleneglycol-mono (chloracetate)  
(n averages 3)*

Chloracetic acid (19 gms. 0.2 mol.) was dissolved in benzene (100 ml.) and boron trifluoride added as the ether complex (1 cc.). Pure ethylene oxide was passed into the solution at such a rate that the temperature did not exceed 40° C. The flow of ethylene oxide was stopped when an increase in weight of 26 gms. was observed (10 hrs.). The excess ethylene oxide, benzene and any dioxane formed during the reaction were evaporated off on the steam bath, finally in vacuo for 1 hr. Yield of colourless oil—44 gms.

In a manner similar to that illustrated above in Examples 1 to 3, other mono- and diesters coming within the scope of general Formulas 1 and 2 can be prepared. By using larger or smaller molar quantities of ethylene oxide than illustrated in Example 3, it is possible to obtain monoesters wherein the value of *n* in general Formula 1 has various values. Likewise by varying the glycol used in the methods described in Examples 1 and 2, it is possible to obtain esters represented by general Formula 2 wherein *n* has various values.

Many of the compounds selected from those represented by the Formulas 1 and 2 above are water soluble. Those compounds which do not have sufficient solubility in water can be dissolved in alcohol solutions, such as ethanol, propanol, etc.

The fog inhibitors which we propose to use are added to the emulsion during the process of manufacture, to avoid loss of sensitivity and to inhibit the growth of fog with passage of time under nonideal conditions of storage.

A solution of the compounds of the invention when added in suitable concentration, before coating, to unsensitized, chemically sensitized, or optically sensitized photographic emulsions does not appreciably affect the sensitometric values for sensitivity and fog when measurements are made soon after coating. When sensitometric measurements are made at appreciable intervals of time, at elevated temperatures and dry or somewhat humid conditions, these compounds do stabilize photographic speed and maintain fog at a low level.

The preparation of silver halide emulsions involves three separate operations: (1) the emulsification and digestion or ripening of the silver halide, (2) the freeing of the emulsion from excess soluble salts, usually by washing, and (3) the second digestion or after-ripening to obtain increased sensitivity. (Mees "The Theory of the Photographic Process," 1942.) We prefer to add the fog-inhibiting agents after the final digestion or after-ripening, although they can advantageously be added prior to digestion.

The photographic emulsions used in practicing our invention are generally of the developing-out type also, it is to be understood that photographic emulsions of varying halide content can advantageously be used. The antifoggant compounds used in our invention have been found particularly useful when employed in conjunction with gelatino-silver bromide emulsions, although they can also be advantageously employed for stabilizing other silver halide emulsions, such as gelatino-silver chloride, bromide, chlorobromide, chlorobromide, etc. The emulsions can be unsensitized, or sensitized with chemical sensitizers or optical sensitizers. Sulfur sensitizers such as those disclosed in Sheppard U. S. Patent 1,574,944 can advantageously be added to the emulsions in the conventional manner. Also, various gold sensitizers can be em-

ployed in the photographic emulsions stabilized according to our invention.

The antifoggant or stabilizing activity of a number of compounds coming within the scope of general Formulas 1 and 2 was determined by incubation of a photographic emulsion at a temperature of 120° F. for three days at a relative humidity of 94% as shown in the table below. The efficiency of the various antifoggants was then evaluated by measuring the speed and fog of the incubated emulsions containing an antifoggant and comparing these measurements with those of the same batch of emulsion before incubation. Also, similar measurements were made on a photographic emulsion containing no antifoggant, both before and after incubation. The tests were made using a high speed silver bromide emulsion exposed on an Eastman type Ib sensitometer with an exposure of  $\frac{1}{50}$  second and then developed for five minutes in a developer of the following composition:

|    |                                | G.    |
|----|--------------------------------|-------|
| 20 | N-methyl-p-aminophenol sulfate | 2.2   |
|    | Hydroquinone                   | 8.8   |
|    | Sodium sulfite (anhydrous)     | 72.0  |
|    | Sodium carbonate (cryst.)      | 130.0 |
| 25 | Potassium bromide              | 4.0   |
|    | Water to make 1 liter.         |       |

TABLE I.—ANTIFOGGANT ACTION

| 30 | Ex.     | Compound | Concentration,<br>g./mol.<br>AgX | Initial Tests |     | 3 days<br>incuba-<br>tion fog |
|----|---------|----------|----------------------------------|---------------|-----|-------------------------------|
|    |         |          |                                  | Speed         | Fog |                               |
| 35 | I(a)    | Blank    |                                  | 100           | .18 | 1.54                          |
|    | I(b)    | A        | 8.5                              | 88            | .12 | .18                           |
| 40 | II(a)   | Blank    |                                  | 100           | .19 | 2.32                          |
|    | II(b)   | B        | 8.5                              | 100           | .15 | 1.43                          |
| 45 | III(a)  | Blank    |                                  | 100           | .19 | 2.32                          |
|    | III(b)  | C        | 4.25                             | 105           | .19 | 1.54                          |
| 50 | IV(a)   | Blank    |                                  | 100           | .21 | 2.37                          |
|    | IV(b)   | D        | 1.7                              | 105           | .18 | 1.97                          |
| 55 | V(a)    | Blank    |                                  | 100           | .16 | 3.50                          |
|    | V(b)    | E        | 0.85                             | 100           | .14 | 1.70                          |
| 60 | VI(a)   | Blank    |                                  | 100           | .34 | 3.52                          |
|    | VI(b)   | F        | 8.5                              | 100           | .20 | 2.85                          |
| 65 | VII(a)  | Blank    |                                  | 100           | .15 | 3.21                          |
|    | VII(b)  | G        | 8.5                              | 75            | .16 | 2.45                          |
| 70 | VIII(a) | Blank    |                                  | 100           | .14 | 3.46                          |
|    | VIII(b) | H        | 8.5                              | 125           | .21 | 3.05                          |
| 75 | IX(a)   | Blank    |                                  | 100           | .08 | 3.16                          |
|    | IX(b)   | J        | 8.5                              | 105           | .09 | 2.30                          |

A=Triethyleneglycol-bis (chloracetate).

B=Triethyleneglycol-bis (β-chloropropionate).

C=Polyethyleneglycol-bis (chloracetate) (n avg. 9).

D=Triethyleneglycol-mono (chloracetate).

E=Ethylene glycol-bis (chloracetate).

F=Triethyleneglycol-bis (trichloroacetate).

G=Triethyleneglycol-mono (bromacetate).

H=Polyethyleneglycol-mono (bromacetate) (n avg. 50).

J=Polyethyleneglycol-mono (iodoacetate) (n avg. 50).

In a manner similar to that illustrated in the above examples, other mono- and diesters selected from those represented by the above general formula can be incorporated in photographic emulsions for the purpose of stabilization. The fog-inhibiting agents useful in practicing our invention can be used in various kinds of photographic emulsions. In addition to being useful in ordinary non-sensitized emulsions, they can also be used in orthochromatic, panchromatic and X-ray emulsions. If used with sensitizing dyes, they can be added to the emulsion before or after the dyes are added. Suitable dispersing agents for the silver halide emulsions stabilized according to our invention comprise gelatin, or other colloids, such as collodion, albumen, cellulose organic derivatives, synthetic resins, etc.

The optimum amount of fog-inhibiting agent can be determined by making the customary tests employed in emulsion making. Of course, the optimum amount for a given emulsion will vary depending on the presence of emulsion addenda, such as chemical sensitizers, optical sensitizers, etc. In general, we have found that from 1.0 g. to 15.0 g. of fog inhibiting agent per mole of silver halide is sufficient for the purpose of our invention.

Instead of adding the fog-inhibiting agent directly to the photographic emulsion, it is sometimes desirable to incorporate the fog-inhibiting agent in a separate layer which is placed in contact with the silver halide emulsion layer which is to be stabilized. Under such conditions, of course, it is advisable to use a higher concentration of fog-inhibiting agent than indicated above. In general, we have obtained excellent results by simply adding a solution of the antifogging agent in a suitable solvent, such as water, ethanol, propanol, etc. directly to the emulsion which is to be stabilized. This method is the one used in Examples I-IX above.

As noted above, certain of the antifogging compounds employed in our invention also have the property of hardening photographic emulsions. This effect for a number of compounds is summarized in the following table wherein the softening temperature of the emulsion containing no antifogging agent is compared with a similar batch of emulsion containing an antifogging agent, the determinations being made before incubation, after three days incubation at 120° F. and a relative humidity of 94%, and after seven days incubation at 120° F. and a relative humidity of 42%. The results are summarized in the following table.

TABLE II.—HARDENING ACTION

| Ex.               | Compound | Concentra-<br>tion, g./<br>mol. AgX | Melting Point, ° F. |        |        |
|-------------------|----------|-------------------------------------|---------------------|--------|--------|
|                   |          |                                     | Initial             | 3 days | 7 days |
| X <sup>(a)</sup>  | Blank    |                                     | 89                  | 104    | 90     |
| X <sup>(b)</sup>  | K        | 4.25                                | 110                 | 170    | 182    |
| XI <sup>(a)</sup> | Blank    |                                     | 91                  | 95     | 88     |
| XI <sup>(b)</sup> | E        | 4.25                                | 153                 | >207   | >207   |
| XII               | L        | 4.25                                | 94                  | 105    | 94     |
| XIII              | G        | 4.25                                | 100                 | 107    | 98     |
| XIV               | M        | 4.25                                | 180                 | 205    | 182    |

K=Polyethyleneglycol-bis (chloracetate) (n avg. 5).  
L=Polyethyleneglycol-mono (chloracetate) (n avg. 6).  
M=Triethyleneglycol-bis (bromacetate).

Tables I and II above show the antifogging activity and hardening action of a number of compounds embraced by our invention. In like manner, other compounds selected from those represented by Formulas 1 and 2 above can be employed to provide the advantages of our invention.

What we claim as our invention and desire secured by Letters Patent of the United States is:

1. A photographic silver halide emulsion containing at least one compound selected from the group consisting of those represented by the following two general formulas:



and



wherein R represents a halogenated alkyl group containing from 1 to 2 carbon atoms and n represents a positive integer.

2. A photographic silver halide emulsion containing at least one compound selected from the group consisting of those represented by the following two general formulas:



and



wherein R represents a halogenated alkyl group containing from 1 to 2 carbon atoms and n represents a positive integer of from 1 to 200.

3. A photographic gelatino-silver halide emulsion con-

taining at least one compound selected from those represented by the following general formula:



wherein R represents a halogenated alkyl group containing from 1 to 2 carbon atoms and n represents a positive integer of from 1 to 200.

4. A photographic gelatino-silver halide emulsion containing at least one compound selected from those represented by the following formula:



wherein R represents a halogenated alkyl group containing from 1 to 2 carbon atoms and n represents a positive integer of from 1 to 200.

5. A photographic gelatino-silver halide emulsion containing at least one compound selected from those represented by the following general formula:



wherein R represents a chlorinated alkyl group containing from 1 to 2 carbon atoms and n represents a positive integer of from 1 to 200.

6. A photographic gelatino-silver halide emulsion containing at least one compound selected from those represented by the following general formula:



wherein R represents a brominated alkyl group containing from 1 to 2 carbon atoms and n represents a positive integer of from 1 to 200.

7. A photographic gelatino-silver bromide emulsion containing at least one compound selected from the group consisting of those represented by the following two general formulas:



and



wherein R represents a halogenated alkyl group containing from 1 to 2 carbon atoms and n represents a positive integer of from 1 to 200.

8. A photographic silver halide emulsion containing at least one compound having the following formula:



9. A photographic silver halide emulsion containing at least one compound having the following formula:



10. A photographic silver halide emulsion containing at least one compound having the following formula:



wherein n has an average value of 9.

11. A photographic silver halide emulsion containing at least one compound having the following formula:



12. A photographic silver halide emulsion containing at least one compound having the following formula:



13. A light-sensitive photographic element comprising a silver halide emulsion layer and an organic colloid layer contiguous to said emulsion layer at least one of said layers containing a compound selected from those represented by the following general formulas:



and



wherein R represents a halogenated alkyl group contain-

ing from 1 to 2 carbon atoms and n represents a positive integer.

References Cited in the file of this patent

UNITED STATES PATENTS

|           |                    |               |
|-----------|--------------------|---------------|
| 2,240,475 | Simmons            | Apr. 29, 1941 |
| 2,356,486 | Weissberger et al. | Aug. 22, 1944 |
| 2,378,203 | Fallesen           | June 12, 1945 |
| 2,441,389 | Blake              | May 11, 1948  |